

No. 877,172.

PATENTED JAN. 21, 1908.

F. M. F. CAZIN.

METHOD OF PRODUCING FILAMENTS FOR ELECTRIC INCANDESCENT LAMPS  
AND THE PRODUCT OF SUCH METHOD.

APPLICATION FILED SEPT. 21, 1904.



WITNESSES:

John T. Schrott

F. C. Gibson

INVENTOR

Francis M. F. Cazin.

BY

Fred G. Detterbeck & Co.  
ATTORNEYS.

# UNITED STATES PATENT OFFICE.

FRANCIS M. F. CAZIN, OF HOBOKEN, NEW JERSEY.

## METHOD OF PRODUCING FILAMENTS FOR ELECTRIC INCANDESCENT LAMPS AND THE PRODUCT OF SUCH METHOD.

No. 877,172.

Specification of Letters Patent.

Patented Jan. 21, 1908.

Application filed September 21, 1904. Serial No. 225,347.

*To all whom it may concern:*

Be it known that I, FRANCIS M. F. CAZIN, of Hoboken, in Hudson county, State of New Jersey, have invented certain new and useful 5 Improvements in the Method of Producing Filaments for Electric Incandescent Lamps and Products of Such Methods, of which the following is a specification.

The purpose of this present application is 10 of the same character and in the same relation to my Patents No. 523,460, of July 24, 1894, and No. 523,461, of same date, and No. 566,285, of August 18, 1896; No. 620,640, of 15 March 7, and Nos. 621,291 and 621,292, of March 14, 1899, No. 640,366 of January 2, 1900, No. 844,778 of Febr. 19, 1907, No. 835,936 of Nov. 13, 1906, No. 786,727 of April 4, 1905, No. 772,215, of Oct. 11, 1904, No. 760,849, of May 24, 1904, No. 770,223 of 20 November 13, 1904 and No. 846,823 of March 12, 1907, and to all the applications therefor as my yet pending applications No. 732,399, No. 3,061, No. 138,084, No. 170,940, No. 183,270, No. 198,564, No. 210,720, No. 210,759, No. 210,870 and No. 220,819—namely, to obtain patent on certain 25 modifications in the processes of manufacturing electric incandescent lamps invented by me and on the lamps that are the products of such manufacture, which processes and lamps were alluded to in these patents, but were not explicitly enough specified and not sufficiently disclosed for formulating on the said specifications and disclosures the 30 proper claims for their protection by patent, though the invention as such or in its essential characteristics has then and there been set forth, and, as conditioned on such identity of purpose and similarity of subject-matter, as 35 well as to facilitate a clear and full understanding of the improvement claimed by this application, I have selected from these my prior applications a few parts to recite, and in special does applicant propose to cite 40 45 50 55 60 65 70 75 80 85 90 95 100 105 110

therefrom the parts, by which he originally disclosed his invention of electrolytic manufacture of electric lamp-filaments or -luminants. (Compare my Patent No. 844,778—page 1 lines 10 to 17 and lines 19 to 37 incl.)

These parts were removed from the specifications, wherein they originally were contained on formal ground, such as division etc.

Having explained in my application No. 655,312 of Oct. 15, 1897 that, which in this 55 connection I considered as my invention—

I formulated thereon the following claims, namely:

“11. An electrolytic apparatus, in which the carbon-filament of an incandescent lamp is attached with its two ends to the negative 60 pole and is surrounded in the bath by a metal-cathode, the form of which is adapted to the loop-form of the filament.

12. The method of electrolytically precipitating a solid coat on a carbon filament, 65 by attaching both ends of the filament to the negative pole of the electrolytic apparatus, immersing the filament-loop into the electrolyte.”

While in these claims the specific “carbon” 70 is mentioned as filament-material applicant has never waived his declaration in his Patent No. 621,291, lines 55, &c., namely: “I have in all of my preceding applications qualified the current passing and 75 resisting filament by function and not by material.” (Compare my Patent No. 621,291, page 1, lines 55, &c.) In corroboration of this my declaration the board of examiners-in-chief in an appeal in the matter of 80 the last-mentioned patent or of the application therefor of October 29, 1895, decided as follows: “The use of a metal filament was not specifically mentioned, although the language used was such as to indicate that 85 applicant’s invention was broad enough to include any material the equivalent of carbon and having the properties indicated.” (Compare my Patent No. 844,778—page 3, lines 40 to 57 incl.) In accordance with 90 such evidence for my conception of that which the filament-core in my electrolytical manufacturing process of electric incandescent filaments must be made of, it is only needed to mention the functional qualities 95 of the selectable material, namely that it be refractory or of high temperature of fusion, be flexible and be electrically conductive, either primarily or when immersed in the electrolyte or when consequent to increased temperature. The filament thus to be manufactured may be described then as consisting of two concentrical parts, or elements, namely a core, such as described as one element and an electrolytic-metallic 105 coating, as the other element, and eventually including a third element, which may be a repeated electrolytic-metallic coating of such metal, as may form with oxygen or with nitrogen a solid compound to include a part 110

of the last-mentioned metal, primarily concentrically on the surface, reacted upon by either oxygen or nitrogen. As a specific metal of the latter class and element I mention titanium. And it should also be understood, that the core-material may by the operation of the lamp, as part of its first manufacture, be partly or entirely absorbed by the coating material.

10 Referring now to the accompanying drawings, in which identical symbols designate the same or equivalent parts Figure 1 is a vertical section of an electric incandescent lamp with the filament indicated in exaggerated thickness and a double-glass-bulb, such as protected by my Patents No. 770,221, 770,222, 770,223 and 846,823, the latter of March 12, 1907, as well as an exclusive glass-base provided with apertures 4, 4 for air-circulation, the same as heretofore described and shown and with a screw-shaped socket-connection-end. Fig. 2. is in exaggerated size, a vertical longitudinal section of a portion of the improved filament, as it 20 would be, if all the mentioned elements were contained in the concentrical coatings thereof, and Fig. 3. is a cross-section thereof, under the same supposition. Fig. 4 is a copy of the illustration of the electrolytic apparatus, indicating the method, as by me claimed under October 15, 1897, and filed on the said date.

25 In the matter of my selection of metals for electrolytical deposition on a conductive core in the shape, that the filament is intended to finally have,—I refer to my Patents No. 835,938 of Nov. 13, 1906 and No. 844,778 of Febr. 19, 1907, and desire it to be understood, that I may use these metals singly or 30 as alloys, and singly or in concentrical layers, as the special purpose of the lamp to be manufactured may call for. The filaments of the by me thus improved electric incandescent lamps then consist of either all or 35 some of the here below described functional parts, namely:

- |    |                                                                                         |                                                                                                                                                                    |
|----|-----------------------------------------------------------------------------------------|--------------------------------------------------------------------------------------------------------------------------------------------------------------------|
| 50 | I. The filament or heated part of the entire conductive element consists mainly of..... | 1. A core for electrolytic deposition, preferably of carbon, and in the shape intended for the lamp-filament when in operation.                                    |
| 55 | II. The protection of part 1. against chemical reaction on its surface.....             | 2. An electrolytically deposited coat on such core, preferably as described and specified in my two Patents No. 835,938 and 844,778.                               |
| 60 | III. A special light-emitting surface of eligible light-emitting efficiency.            | 3. An electrolytically deposited or coat of metal, the oxygen or nitrogen compound of which is a solid, and when metal has but normal affinity for either or both. |
|    |                                                                                         | 4. A surface of a metal-compound, the result of chemical reaction on the surface-metal.                                                                            |

As shown in my application, as first filed in this case, I intended to explain in detail 65 my understanding of every expression, used in the preceding table as well as to show by the science of chemistry the practicability of electrolytically depositing the single metals or the alloys of metals, and by the art of 70 electrolytic deposition or plating the practi-

cability of doing so in even and adhering single or concentrical plural coats.—But, since those skilled in the chemical and electrolytical art, will be able to manufacture my improved metallized or metal-filaments as by 75 me specified and by the method by me claimed, after this method as such has by me been invented and disclosed,—I prefer now to desist from all further detail-explanations.

Having thus described my invention, what 80 I claim and desire to secure by Letters Patent, is:—

1. The method of manufacturing filaments for electric incandescent lamps, which consists in using a filament-core, bent in the 85 linear shape, that the finished filament is intended to have, as one of the electrodes in an electrolytic plating apparatus, and coating the said core in the electrolyte-bath of the said apparatus with metal by the application 90 of electric current, passing between electrodes through the electrolyte.

2. The method of manufacturing filaments for electric incandescent lamps, which consists in using a filament-core, bent in the 95 linear shape, that the finished filament is intended to have, as one of the conductive electrodes in an electrolytic plating-apparatus, and coating the said core in electrolyte-baths of different chemical composition, applied successively in such apparatus, with concentrical layers of metal by the application of electric current, passing between electrodes through the different electrolytes, 100 to which the core-electrode is exposed successively.

3. The method of manufacturing lumi-nants for electric incandescent lamps, which consists in using a conductive filament-core, bent in the linear longitudinal shape, that 110 the finished filament is intended mainly to have,—as one of the electrodes in some electrolytic plating apparatus,—and coating the said core in electrolyte-baths of different chemical composition and adequate temperature,—successively applied in such apparatus,—with concentrical layers of metallic alloys, by the application of adequate electric current, passing between electrodes through the different electrolytes successively.

4. The method of manufacturing filaments for electric incandescent lamps, which consists in using a conductive filament-core, bent into the main longitudinal linear shape, that is intended for the finished filament,—as one of the electrodes in some electrolytic plating apparatus,—and coating the said core successively in different electrolyte-baths of adequate chemical composition, with different concentrical metallic layers, and applying to the coated filament electric adequate operative current, allowing such chemical inter-reaction and reaction on the surface-coat, as will take place under such 135

current in eventual completion of the filament for adequate use.

5. A filament in an electric incandescent lamp primarily consisting of a conductive core, coated, when longitudinally bent into its final and main filament-shape, with an electrolytic metal-cover.

6. A filament in an electric incandescent lamp, which filament consists primarily of a 10 conductive core, bent longitudinally into the final shape of the filament mainly, which core is coated with an electrolytic metal-plating, which plating consists of several concentrical layers.

15 7. A filament in an electric incandescent lamp, which filament consists primarily of a conductive core, primarily bent longitudinally into the main filament-shape, intended for the finished filament,—which core in such 20 shape is coated with electrolytic metal-alloy-plating in different concentrical layers.

8. A filament in an electric incandescent lamp, which filament primarily consists of a conductive, preferably carbon-core, pri-

marily and mainly bent longitudinally into 25 the final filament-shape,—which core in such shape has a cover of electrolytical metal-plating in concentrical layers and has by subjecting the same to an adequate electric current, passing from end to end, been exposed 30 to chemical reaction and inter-reaction between constituents and on its surface under adequate conditions of current and surroundings.

9. A filament in an electric incandescent 35 lamp, which luminant consists primarily of a conductive core, bent longitudinally into the main shape intended for the completed lum- 40 inant,—which core in such shape is coated with electrolytic metal-plating in concentrical layers, the one on the surface containing titanium, subjected to chemical reaction by a longitudinally passing electric current under adequate conditions and surroundings.

FRANCIS M. F. CAZIN.

Witnesses:

MINNA E. CAZIN,  
N. W. WREN.